

## UNITED STATES PATENT OFFICE

2,523,100

MINERAL OIL COMPOSITION AND  
ADDITIVE THEREFOR

Lawrence T. Eby, Roselle, N.J., assignor to Standard Oil Development Company, a corporation of Delaware

No Drawing, Application May 17, 1947,  
Serial No. 748,855

11 Claims. (Cl. 252—47.5)

1

This invention relates to new chemical products and to improved lubricating oils containing such products as additives.

Many types of chemical compounds have been proposed for use as detergent additives for lubricating oils, for the purpose of dispersing sludge and maintaining a clean engine condition when such oils are employed as crankcase lubricants for internal combustion engines. Most of the additives which have been found effective for such use contain metals, and while their sludge dispersing properties are satisfactory, there is the objection that a metal-containing deposit will be formed which gradually becomes forced into the engine cylinder and tends to foul the spark plugs and produce other undesirable effects. It is accordingly an object of the present invention to provide an additive which is an effective detergent and at the same time contains no metal and is accordingly entirely free from any tendency to form a deposit of the type described.

The new class of additives which are described herein are non-metallic and have been found to possess the required degree of sludge dispersing and detergent properties, and these have been found to possess in addition the property of inhibiting oxidation of the oil. They have also been found to be valuable additives for extreme pressure lubricants containing chlorine compounds which tend to evolve hydrogen chloride during storage, the additive having the effect of neutralizing such corrosive products without at the same time producing an objectionable precipitate during periods of storage of a lubricant.

The new additives of the present invention, which are also new chemical compounds, are quaternary bases and salts formed by the alkylation of dialkylaminomethyl phenol sulfides containing certain oil-solubilizing alkyl groups, as specified hereinafter. The new additives may be defined broadly by the formulas



and



in which R<sub>1</sub>, R<sub>2</sub> and R<sub>3</sub> are alkyl radicals with a total of at least 9 carbon atoms, X is a hydroxyl group or an inorganic or organic acid radical, R<sub>4</sub> is hydrogen or an alkyl radical, R and R' are alkyl radicals, each containing at least

4 and preferably 8 carbon atoms, and n is a number from 1 to 4. The acid radicals which may be substituted for the hydroxyl groups of such quaternary bases may be any acid radicals, whether inorganic or organic. The acid radicals which have been found to be particularly desirable for the purpose of the present invention and which may be readily introduced into the compounds are those which are derived from the following acids: phosphoric, thiophosphoric, carbonic, thiocarbonic, sulfurous, sulfuric, mono-alkyl sulfuric, tetraisobutetyl sulfonic, thiocyanic, hydrochloric, nitric and boric.

In the preparation of the new compounds and additives of the present invention, alkylated phenols are first formed by reacting phenols with olefins in the presence of an alkylating catalyst. From these the monosulfides and polysulfides may be formed by reaction with chlorides of sulfur. The aminoalkyl derivatives of such products may be formed by first preparing an alkylaminoalkyl-alkyl ether and then reacting the same in the presence of an alcohol with the alkylated phenol sulfide. From the products thus formed a quaternary ammonium base may be derived by treating with an alkylating agent, such as a dialkyl sulfate or an alkyl halide, followed by reaction with a free base. As an alternative method, the alkyl phenol sulfide may first be converted into a chloralkyl derivative by reaction with an aldehyde in the presence of hydrogen chloride, further reacting the product thus formed with a tertiary amine, and finally reacting the resulting chlorinated compound with a base. If it is desired to convert the base into a salt, the former may be reacted with an acid or with an acid anhydride. Phosphoric or thiophosphoric acid salts may thus be formed by reaction with an oxide or sulfide of phosphorus. Similarly, a thiocarbonate salt may be formed by reaction with carbon disulfide. The preparation of a number of specific examples of the compounds of the present invention is described in detail below.

The quantity of the additives of the present invention which is most advantageously blended in the mineral lubricating oil will depend upon the property of the additive which it is most desired to exploit. When employed for detergent and sludge dispersing purposes, the quantity most suitable will generally vary from 1 to 5%. For merely inhibiting bearing corrosion and the like the quantity most desirable will be from 0.05% to 2%. When the additive is to be employed as a corrosion inhibitor in an extreme pressure lubricant composition, it is desirable to employ from 0.2% to 1%, particularly when the lubricating oil contains about 10% of a chlorinated hydrocarbon containing approximately 32% chlorine.

The preparation and testing of a number of examples of the compounds of the present invention are illustrated by the examples to be described in detail below, but such examples are not to be construed as limiting the scope of the invention in any manner.

**Example 1.—Di(di-n-octylmethylaminomethyl)-tert-octylphenol polysulfide hydroxide**

In a flask was placed 200 cc. of absolute ethyl alcohol, 120.5 g. (0.5 mol) of di-n-octylamine and 15 g. (0.5 mol CH<sub>2</sub>O) of trioxymethylene. The mixture was stirred overnight to give a solution of 0.5 mol of di-n-octylaminomethyl ethyl ether.

A solution of 1030 g. (5 mols) of distilled tert-octylphenol and 1000 cc. of chloroform was charged to a flask and stirred while 770 g. (7.5 mols) of sulfur dichloride was added during 2½ hours, keeping the temperature below 30° C. The mixture was refluxed with stirring for 3 hours and then cooled, poured into water, extracted with ether, washed free of hydrochloric acid, dried over sodium sulfate, and the solvent removed by distillation, finishing at reduced pressure. The residue weighed 1506 g. and contained 15.61% sulfur (Parr Bomb), which corresponds to the formula



Half of the solution (0.25 mol) of di-n-octylaminomethyl ethyl ether described above was added to a solution of 49.3 g. (0.102 mol) of the sulfurized phenol described above in 200 cc. of absolute ethyl alcohol. The mixture was stirred and refluxed overnight. After cooling, 63 g. (0.5 mol) of dimethylsulfate was added and the mixture stirred overnight. The volatile constituents were removed by vacuum distillation, finishing over a boiling water bath at 2 mm. pressure. The residue weighing 173 g. was a brown viscous liquid which was found to contain 13.30% sulfur (Parr Bomb) and 1.95% nitrogen (Kjeldahl).

This di(di-n-octylmethylaminomethyl)-tert-octylphenol polysulfide di(methyl sulfate) was dissolved in ether and stirred with 10% aqueous sodium hydroxide overnight. The ether layer was separated, washed with water, dried over anhydrous potassium carbonate, filtered, and the ether removed by distillation. The residue was a brown liquid less viscous than the methyl sulfate and contained 5.29% sulfur and 3.00% nitrogen. The product is di(di-n-octylmethylaminomethyl)-tert-octylphenol polysulfide hydroxide.

**Example 2.—Di-n-octylmethylaminomethyl-tert-octylphenol polysulfide hydroxide**

The same procedure as that used in Example 1 was used, except that 98.5 g. (0.204 mol) of the alkylated phenol polysulfide was used. The di-n-octylmethylaminomethyl-tert-octylphenol polysulfide was obtained as a brown viscous liquid weighing 217.2 g. and containing 13.73% sulfur and 1.53% nitrogen. The free base was obtained by reacting such product with sodium hydroxide solution as in Example 1, and was obtained as a brown viscous liquid not as viscous as the sulfate and containing 7.22% sulfur and 2.15% nitrogen.

**Example 3.—Thiophosphate of di(di-n-octylmethylaminomethyl)-tert-octylphenol polysulfide hydroxide**

1030 g. (5 mols) of distilled tert-octylphenol and 1 l. of chloroform were placed in a flask equipped with stirrer, dropping funnel, return condenser and thermometer. 386 g. (3.75 mols) of sulfur dichloride was dropped into the mixture while stirring over a period of 6 hours, keeping the temperature below 30° C. The mixture was refluxed 6 hours, cooled and poured into water. The organic layer was removed, washed again with water and dried over anhydrous sodium sulfate. The mixture was filtered from the drying agent and stripped of solvent by vacuum distillation. The residue was a reddish brown resin-like solid when cooled and weighed 1081.7 g. The product contained 10.69% sulfur and thus corresponds approximately to the formula



228.8 g. (0.5 mol) of the phenol sulfide product described above, 600 cc. of absolute ethyl alcohol, 241 g. (1 mol) of di-n-octylamine and 30 g. (1 mol CH<sub>2</sub>O) of trioxymethylene were stirred together for one hour and then refluxed for one hour. The mixture was cooled to room temperature and 163.8 g. (1.3 mols) of dimethyl sulfate was added with stirring to produce a solution of di(di-n-octylmethylaminomethyl)-tert-octylphenol polysulfide di-(methyl sulfate).

225 cc. of 25% of aqueous sodium hydroxide solution and 275 cc. of water were added to the alcohol solution of di(di-n-octylmethylaminomethyl)-tert-octylphenol polysulfide di-(methyl sulfate) described above. The mixture was stirred for 3 hours. The organic material was extracted with 100 cc. of ether after dilution with 1 l. of water. The ether extract was stirred with 100 cc. of 25% aqueous sodium hydroxide solution and 100 cc. water for 3 hours. The organic layer was washed with three 500 cc. portions of water and dried over anhydrous potassium carbonate. After filtering, the volatile materials were removed by vacuum distillation, leaving 463.1 g. of brown viscous liquid residue which contained 4.86% sulfur and 2.61% nitrogen.

51.35 g. (0.05 mol) of di(di-n-octylmethylaminomethyl)-tert-octylphenol sulfide hydroxide, prepared as described in the preceding paragraph, and 3.53 g. (0.0167 mol) of P<sub>2</sub>S<sub>5</sub> were stirred together at room temperature for 20 hours. Hydrogen sulfide was liberated. 50 cc. of ether was added and the mixture stirred 24 hours. The ether was removed by distillation leaving a viscous dark reddish brown material containing 8.25% sulfur, 2.37% nitrogen, and 1.88% phosphorus. The product is thus a thiophosphate of di(di-n-octylmethylaminomethyl)-tert-octylphenol polysulfide hydroxide.

**Example 4.—Thiophosphate of di(di-n-octylmethylaminomethyl)-tert-octylphenol polysulfide hydroxide**

51.35 g. (0.05 mol) of di(di-n-octylmethylaminomethyl)-tert-octylphenol polysulfide hydroxide, prepared as described in Example 3, and 5.3 g. (0.025 mol) of P<sub>2</sub>S<sub>5</sub> were stirred together at room temperature for 20 hours. Hydrogen sulfide was liberated. 50 cc. of ether was added and the mix-

ture stirred 24 hours. The ether was removed by distillation, leaving a viscous dark reddish brown material containing 8.83% sulfur, 2.24% nitrogen and 1.97% phosphorus.

*Example 5.—Thiocarbonate of di(di-n-octylmethylaminomethyl)-tert-octylphenol polysulfide hydroxide*

51.35 g. (0.05 mol) of di(di-n-octylmethylaminomethyl)-tert-octylphenol polysulfide hydroxide, prepared as described in Example 3, and 25 cc. of carbon bisulfide were stirred together for 20 hours. There was no apparent liberation of hydrogen sulfide, but a homogeneous solution formed with a rise in temperature of 3° C. The solution was diluted with 50 cc. of ether and then stripped of volatile constituents by vacuum distillation over a boiling water bath. The residue, weighing 51.2 g. was a reddish brown viscous liquid which contained 6.49% sulfur and 2.58% nitrogen. The product is thus a thiocarbonate of di(di-n-octylmethylaminomethyl)-tert-octylphenol polysulfide hydroxide.

*Example 6.—Diocetyl methylaminomethyl-tert-octylphenol polysulfide methyl sulfate*

1030 g. (5 mols) of distilled tert-octylphenol and 1 l. of chloroform were placed in a flask equipped with stirrer, dropping funnel, return condenser and thermometer. 386 g. (3.75 mols) of sulfur dichloride was dropped into the mixture with stirring over 6 hours, keeping the temperature below 30° C. The mixture was refluxed 4 hours, cooled and poured into water. The organic layer was removed, washed again with water, and then dried over anhydrous sodium sulfate. The mixture was filtered from the drying agent and stripped of solvent by vacuum distillation. The residue was a reddish brown resin-like solid weighing 1155 g. and containing 10.69% sulfur, which corresponds approximate to the formula



228.5 g. (0.5 mol) of the product described above was dissolved in 600 cc. of absolute ethyl alcohol and placed in a flask equipped with a dropping funnel. A solution of 120.5 g. (0.5 mol) of di-n-octylamine and 15 g. (0.5 mol CH<sub>2</sub>O) of trioxymethylene in 200 cc. of absolute ethyl alcohol was added slowly from the dropping funnel. The mixture was refluxed overnight. After cooling, 126 g. (1 mol) of dimethyl sulfate was added slowly with stirring. The mixture was stripped of volatile components by vacuum distillation and the residue was the brown very viscous liquid weighing 509.9 g. and containing 11.36% sulfur and 1.40% nitrogen. The product was thus di-n-octylmethylaminomethyl-tert-octylphenol polysulfide methyl sulfate.

*Example 7.—Di(di-n-octylmethylaminomethyl)-tert-octylphenol polysulfide di(methyl sulfate)*

Example 6 was repeated except that 114.3 g. (0.25 mol) of the polysulfide product was used. The product was a very viscous brown liquid weighing 356.1 g. and containing 11.62% sulfur and 1.87% nitrogen. The product is di(di-n-octylmethylaminomethyl)-tert-octylphenol polysulfide di(methyl sulfate).

*Example 8.—Di-n-octylmethylaminomethyl-tert-octylphenol polysulfide hydroxide*

374.2 g. of the product from Example 6 and 350 cc. of ether were placed in a flask and stirred with 250 cc. of 20% aqueous sodium hydroxide solution. After stirring for 1.5 hours, the layers were allowed to separate and the ether layer again stirred with 20% aqueous sodium hydroxide solution. The layers were separated and the ether solution washed twice with water and then allowed to stand overnight to separate any residual water in the organic layer. The volatile constituents were removed from the organic layer by vacuum distillation. The residue was a brown viscous liquid weighing 290.5 g. and containing 6.54% sulfur and 1.88% nitrogen. This product was di-n-octylmethylaminomethyl-tert-octylphenol polysulfide hydroxide.

*Example 9.—Di(di-n-octylmethylaminomethyl)-tert-octylphenol polysulfide hydroxide*

299.4 g. of the product from Example 7 and 300 cc. of ether were placed in a flask and stirred with 200 cc. of 20% aqueous sodium hydroxide solution. After stirring for 1½ hours the layers were allowed to separate and the ether layer again stirred with 20% aqueous sodium hydroxide solution. The layers were separated and the ether solution washed twice with water, dried over anhydrous potassium carbonate and stripped of volatile constituents by vacuum distillation. The residue was a brown viscous liquid weighing 198.8 g. and containing 4.99% sulfur and 2.70% nitrogen. This product was di(di-n-octylmethylaminomethyl)-tert-octylphenol polysulfide hydroxide.

*Example 10.—Di-n-butylmethylaminomethyl-tert-butylphenol sulfide hydroxide*

40 A glass reaction flask was charged with 300.4 g. (2.0 mols of p-tert-butylphenol and 500 ml. of chloroform. The mixture was stirred and 103.0 g. (1.0 mols) of sulfur dichloride was added from a dropping funnel over three hours while maintaining the temperature below 30° C. The solution was heated under reflux for four hours, cooled, washed with water, then with aqueous sodium bicarbonate solution and dried over sodium sulfate. The drying agent was removed by filtration and the organic layer stripped of solvent by distillation to a temperature of 115° C. at 1 mm. pressure. The residue was p-tert-butylphenol sulfide.

45 A glass reaction flask was charged with 148.7 g. (0.450 mol) of tert-butylphenol sulfide (prepared as described above) and 400 ml. of absolute ethyl alcohol. A solution of 15.0 g. (0.5 mol CH<sub>2</sub>O) of trioxymethylene, 200 ml. of absolute ethyl alcohol, and 65.1 g. of di-n-butylamine was added to the flask and stirred for one-half hour. The solution was heated under reflux for four hours. The solution was cooled and 126 g. (1 mol) of dimethyl sulfate was added after which the mixture was stirred for an additional two hours before stripping to remove unreacted reagents and solvent. Stripping was carried to 100° C. at 2 mm. pressure to obtain 342.7 g. of residue, which is di-n-butylaminomethyl-tert-butylphenol sulfide methyl sulfate. This product was not soluble in 1% concentration in either a 100 V. I. or 28 V. I. mineral lubricating (S. A. E. 20) oil.

50 A glass flask was charged with 119.8 g. (0.205 mol) of di-n-butylmethylaminomethyl-tert-butylphenol sulfide methyl sulfate (prepared as de-

scribed above), 200 ml. of benzene, and 100 ml. of aqueous 25% sodium hydroxide solution. The mixture was stirred for 1.5 hours and the aqueous layer then removed. Another 100 ml. of 25% sodium hydroxide was added and the mixture stirred for 1.5 hours. The organic layer was washed twice with distilled water. The second wash required centrifuging to remove the water. The organic layer was stripped to a temperature of 100° C. at 1 mm. The residue weighed 72.0 g. and was not completely soluble in the 100 V. I. S. A. E. 20 oil but the 1% solution in the 28 V. I. oil was clear at room temperature. The residue was di-n-butylmethylaminomethyl-tert-butylphenol sulfide hydroxide.

*Example 11.—Carbon black dispersion tests*

A series of carbon black dispersion tests were carried out, as described in U. S. Patent 2,390,342, to measure the comparative effectiveness of the additives of the present invention as agents for dispersing sludge in lubricating oil. In these tests 6% by weight of activated carbon was added to the oil blend containing the additive and thoroughly dispersed in the oil by stirring with an "egg beater" type mixer for 15 minutes while the temperature of the oil was maintained at 250° F. 250 cc. of the blend was then placed in a 250 cc. graduated cylinder and allowed to settle for 24 hours while the temperature was maintained at 200° F. If an additive is not a dispersing agent, the carbon black settles rapidly at this point leaving clear oil at the top in an hour or two. A very effective disperser will maintain the carbon black in suspension so that no change in the opaque slurry is apparent even after a 24-hour period. With all but the most potent dispersing agents stratification occurs with a black layer at the bottom (high concentration of carbon black) and a blue opaque layer at the top (reduced carbon black concentration). Cases of this type, known as "blue line" separations, are only detectable in reflected light and the top oil contains smaller particles of dispersed carbon black. Base oil A used in this test was a paraffinic oil of S. A. E. 20 grade, while base oil B was a naphthenic oil of 55 seconds viscosity Saybolt at 210° F. The results of the test when applied to blends containing the products of Examples 1, 2, and 10 are shown in the following table, in which the results are shown as the volume of oil below the line of demarcation and containing essentially all of the dispersed carbon black after the settling period.

| Additive                                                                                            | Cc. Oil Containing Dispersed Carbon Black                |
|-----------------------------------------------------------------------------------------------------|----------------------------------------------------------|
| Base Oil A.                                                                                         |                                                          |
| Base oil A+1% di-(di-n-octyl-methylaminomethyl)-tert-octylphenol polysulfide hydroxide (Example 1). | 87 (top oil is clear).<br>234 ("blue line" separation).  |
| Base oil A+1% di-n-octyl-methylaminomethyl-tert-octylphenol polysulfide hydroxide (Example 2).      | 182 ("blue line" separation).                            |
| Base oil B.                                                                                         |                                                          |
| Base oil B+1% di-n-butyl-methylaminomethyl-tert-butylphenol sulfide hydroxide (Example 10).         | 115 (top oil is clear).<br>134 ("blue line" separation). |

*Example 12.—Bearing corrosion tests*

Blends of the products of Examples 3, 4 and 5 in a lubricating oil base were submitted to a corrosion test designed to measure the effectiveness of the products in inhibiting the corrosiveness of a typical mineral lubricating oil toward the surfaces of copper-lead bearings. The base oil employed was a paraffinic type mineral

lubricating oil of S. A. E. 20 grade. The test was applied to the unblended base oil as well as to the blends. The test was conducted as follows: 500 cc. of the oil was placed in a glass oxidation tube (13 inches long and 2½ inches in diameter) fitted at the bottom with a ¼ inch air inlet tube perforated to facilitate air distribution. The oxidation tube was then immersed in a heating bath so that the oil temperature was maintained at 325° F. during the test. Two quarter sections of automotive bearings of copper-lead alloy of known weight having a total area of 25 sq. cm. were attached to opposite sides of a stainless steel rod which was then immersed in the test oil and rotated at 600 R. P. M., thus providing sufficient agitation of the sample during the test. Air was then blown through the oil at the rate of 2 cu. ft. per hour. At the end of each 4-hour period the bearings were removed, washed with naphtha and weighed to determine the amount of loss by corrosion. The bearings were then repolished (to increase the severity of the test), reweighed, and then subjected to the test for additional 4-hour periods in like manner. The results are given in the following table as "corrosion life," which indicates the number of hours required for the bearings to lose 100 mg. in weight, determined by interpolation of the data obtained in the various periods.

| Oil Blend                          | Bearing Corrosion Life, hrs. |
|------------------------------------|------------------------------|
| Base Oil                           | 6                            |
| Base Oil+0.5% Product of Example 3 | 13                           |
| Base Oil+0.5% Product of Example 4 | 16                           |
| Base Oil+0.5% Product of Example 5 | 10                           |

*Example 13.—Extreme pressure lubricant corrosion and stability tests*

The ability of the additives of the present invention to prevent corrosion due to the extreme pressure agent of an extreme pressure lubricant was tested by incorporating 0.4% of each of several examples of such additives in an extreme pressure lubricant consisting of 90% of an acid and clay treated Coastal oil distillate having a viscosity of 70 seconds Saybolt at 210° F. and 10% of an extreme pressure lubricant consisting of a sulfurized and chlorinated kerosene containing 6 to 7% sulfur and about 32% chlorine, and testing such blends in an S. A. E. Extreme Pressure Testing Machine. The machine was operated for 30 seconds at 20 pounds load and then at 50 pounds load for 5 minutes. The test ring was placed in a desiccator containing a saturated solution of sodium carbonate for 24 hours, washed with benzene and observed for evidence of corrosion. The amount of corrosion is given as the percentage of the entire area which showed corrosion.

Results are as follows:

| Amount of Corrosion (Average of 2 Rings)                                                      | Per cent |
|-----------------------------------------------------------------------------------------------|----------|
| Blank                                                                                         | 85       |
| Diocetylaminomethyl-tert-octylphenol polysulfide methyl sulfate (Example 6)                   | 25       |
| Di-(di-n-octylmethylaminomethyl)-tert-octylphenol polysulfide di-(methyl sulfate) (Example 7) | 10       |
| Diocetylaminomethyl-tert-octylphenol polysulfide hydroxide (Example 8)                        | 18       |
| Di-(di-n-octylmethylaminomethyl) tert-octylphenol hydroxide (Example 9)                       | 30       |

The stability of an extreme pressure lubricant in the presence of the corrosion preventing additives of the present invention was tested by first preparing an extreme pressure agent described above containing 4% of an additive of the present invention, then storing such concentrate in a glass vessel in the presence of a steel strip for 24 hours at 150° F., after which the material was cooled and blended in 10% portions in a base stock consisting of a Panhandle bright stock, which is a highly paraffinic oil, and observing the condition of the oil after 10 days' storage at room temperature. Blends prepared with dioctylmethylaminomethyl-tert-octylphenol polysulfide methyl sulfate and with dioctylmethylaminomethyl-tert-octylphenol polysulfide hydroxide, the same being two of the additives tested for corrosion preventing ability in this example, showed the additives to be completely soluble after the storage period.

The products of the present invention may be employed not only in ordinary hydrocarbon lubricating oils but also in the "heavy duty" type of lubricating oils which have been compounded with such detergent type additives as metal soaps, metal petroleum sulfonates, metal phenates, metal alcoholates, metal alkyl phenol sulfides, metal organo phosphates, thiophosphates, phosphites and thiophosphites, metal salicylates, metal xanthates and thioxanthates, metal thiocarbamates, amines and amine derivatives, reaction products of metal phenates and sulfur, reaction products of metal phenates and phosphorus sulfides, metal phenol sulfonates, and the like. Thus, the additives of the present invention may be used in lubricating oils containing such other addition agents as barium tert-octylphenol sulfide, calcium tert-amylphenol sulfide, nickel oleate, barium octadecylate, calcium phenyl stearate, zinc diisopropyl salicylate, aluminum naphthenate, calcium cetyl phosphate, barium di-tert-amylphenol sulfide, calcium petroleum sulfonate, zinc methyl cyclohexyl thiophosphate, calcium dichlorostearate, etc. Other types of additives, such as phenols and phenol sulfides may also be employed.

The lubricating oil base stocks used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The oils may be refined by conventional methods using acid, alkali and/or clay or other agents such as aluminum chloride, or they may be extracted oils produced, for example, by solvent extraction with solvents of the type of phenol, sulfur dioxide, furfural, dichlorodimethyl ether, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coil tar fractions and coal tar or shale oil distillates may also be used. Also, for special applications, animal, vegetable or fish oils or their hydrogenated or voltalized products may be employed in admixture with mineral oils.

For the best results the base stock chosen should normally be that oil which without the new additive present gives the optimum performance in the service contemplated. However,

since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additive, although in some cases auxiliary solvent agents may be used. The lubricating oils, however they may have been produced, may vary considerably in viscosity and other properties depending upon the particular use for which they are desired, but they usually range from about 40 to 150 seconds Saybolt viscosity at 210° F. For the lubricating of certain low and medium speed Diesel engines the general practice has often been to use a lubricating oil base stock prepared from naphthenic or aromatic crudes and having a Saybolt viscosity at 210° F. of 45 to 90 seconds and a viscosity index of 0 to 50. However, in certain types of Diesel engine and other gasoline engine service, oils of higher viscosity index are often preferred, for example, up to 75 to 100, or even higher, viscosity index.

In addition to the materials to be added according to the present invention, other agents may also be used such as dyes, pour depressors, heat thickened fatty oils, sulfurized fatty oils, organo-metallic compounds, metallic or other soaps, sludge dispersers, antioxidants, thickeners, viscosity index improvers, oiliness agents, resins, rubber, olefin polymers, voltalized fats, voltalized mineral oils, and/or voltalized waxes and colloidal solids such as graphite or zinc oxide, etc. Solvents and assisting agents, such as esters, ketones, alcohols, aldehydes, halogenated or nitrated compounds, and the like may also be employed.

Assisting agents which are particularly desirable as plasticizers and defoamers are the higher alcohols having eight or more carbon atoms and preferably 12 to 20 carbon atoms. The alcohols may be saturated straight and branched chain aliphatic alcohols such as octyl alcohol ( $C_8H_{17}OH$ ), lauryl alcohol, ( $C_{12}H_{25}OH$ ), cetyl alcohol ( $C_{16}H_{33}OH$ ), stearyl alcohol, sometimes referred to as octadecyl alcohol ( $C_{18}H_{37}OH$ ), heptadecyl alcohol ( $C_{17}H_{35}OH$ ), and the like, the corresponding olefinic alcohols such as oleyl alcohol; cyclic alcohols such as naphthenic alcohols; and aryl substituted alkyl alcohols, for instance, phenyl octyl alcohol, or octadecyl benzyl alcohol or mixtures of these various alcohols, which may be pure or substantially pure synthetic alcohols. One may also use mixed naturally occurring alcohols such as those found in wool fat (which is known to contain a substantial percentage of alcohols having about 16 to 18 carbon atoms) and in sperm oil (which contains a high percentage of cetyl alcohol); and although it is preferable to isolate the alcohols from those materials, for some purposes, the wool fat, sperm oil or other natural products rich in alcohols may be used per se. Products prepared synthetically by chemical processes may also be used, such as alcohols prepared by the oxidation of petroleum hydrocarbons, e. g., paraffin wax, petrolatum, etc.

In addition to being employed in crankcase lubricants the additives of the present invention may also be used in extreme pressure lubricants, engine flushing oils, industrial oils, general machinery oils, process oils, rust preventive compositions and greases.

The antioxidant or stabilizing additives of the present invention may be employed not only in mineral lubricating oils, but also in hydrocarbon products generally, where improved resistance to oxidation is desired. Thus, the products may be added to motor oils, Diesel fuels, kerosene, waxes, hydrocarbon polymers, natural and synthetic rubbers, etc.

The present invention is not to be considered as limited by any of the examples described herein, which are given by way of illustration only, but is to be limited solely by the terms of the appended claims.

I claim:

1. A composition consisting essentially of a hydrocarbon base containing 0.05 to 5% of a compound of the formula



wherein R and R' are alkyl radicals each containing at least 4 carbon atoms, n is a number from 1 to 4, and wherein there is attached to the benzene nuclei one to two radicals, not more than one such radical to a given benzene nucleus, of the formula



wherein R<sub>1</sub>, R<sub>2</sub>, and R<sub>3</sub> are alkyl radicals containing an overall total of at least 9 carbon atoms and X is a member of the group consisting of hydroxyl radicals and acid radicals derived from water-soluble acids having an ionization constant at least as great as  $3.5 \times 10^{-7}$ .

2. A mineral lubricating oil containing 0.05 to 5% of a compound of the formula



wherein R and R' are alkyl radicals each containing at least 4 carbon atoms, n is a number from 1 to 4, and wherein there is attached to the benzene nuclei one to two radicals, not more than one such radical to a given benzene nucleus, of the formula



wherein R<sub>1</sub>, R<sub>2</sub>, and R<sub>3</sub> are alkyl radicals containing an overall total of at least 9 carbon atoms and X is a member of the group consisting of hydroxyl radicals and acid radicals derived from water-soluble acids having an ionization constant at least as great as  $3.5 \times 10^{-7}$ .

3. A mineral lubricating oil composition ac-

cording to claim 2 in which X of the formula is OH, and R and R' are each C<sub>8</sub>H<sub>17</sub>.

4. A mineral lubricating oil composition according to claim 2 in which X of the formula is OH, R<sub>1</sub>, R<sub>2</sub>, R, and R' are each C<sub>8</sub>H<sub>17</sub>, and R<sub>3</sub> is CH<sub>3</sub>.

5. A mineral lubricating oil composition according to claim 2 in which X is a thiophosphate radical, R<sub>1</sub>, R<sub>2</sub>, R, and R' are each C<sub>8</sub>H<sub>17</sub>, and R<sub>3</sub> is CH<sub>3</sub>.

6. A mineral lubricating oil composition according to claim 2 in which X is a thiocarbonate radical, R<sub>1</sub>, R<sub>2</sub>, R, and R' are each C<sub>8</sub>H<sub>17</sub>, and R<sub>3</sub> is CH<sub>3</sub>.

7. As a new compound a compound of the formula

20



wherein R and R' are alkyl radicals each containing at least 4 carbon atoms, n is a number from 1 to 4, and wherein there is attached to the benzene nuclei one to two radicals, not more than one such radical to a given benzene nucleus, of the formula

30



wherein R<sub>1</sub>, R<sub>2</sub>, and R<sub>3</sub> are alkyl radicals containing an overall total of at least 9 carbon atoms, and X is a member of the group consisting of hydroxyl radicals and acid radicals derived from water-soluble acids having an ionization constant at least as great as  $3.5 \times 10^{-7}$ .

8. A compound according to claim 7 in which X of the formula is OH, and R and R' are each C<sub>8</sub>H<sub>17</sub>.

9. A compound according to claim 7 in which X is OH, R<sub>1</sub>, R<sub>2</sub>, R and R' are each C<sub>8</sub>H<sub>17</sub>, and R<sub>3</sub> is CH<sub>3</sub>.

10. A compound according to claim 7 in which X is a thiophosphate radical, R<sub>1</sub>, R<sub>2</sub>, R and R' are each C<sub>8</sub>H<sub>17</sub>, and R<sub>3</sub> is CH<sub>3</sub>.

11. A compound according to claim 7 in which X is a thiocarbonate radical, R<sub>1</sub>, R<sub>2</sub>, R, and R' are each C<sub>8</sub>H<sub>17</sub>, and R<sub>3</sub> is CH<sub>3</sub>.

LAWRENCE T. EBY.

#### REFERENCES CITED

The following references are of record in the file of this patent:

#### UNITED STATES PATENTS

| Number    | Name              | Date          |
|-----------|-------------------|---------------|
| 2,218,739 | Bruson            | Oct. 22, 1940 |
| 2,260,967 | Bruson            | Oct. 28, 1941 |
| 2,334,594 | Zimmer et al.     | Nov. 16, 1943 |
| 2,345,239 | Cook et al.       | Mar. 28, 1944 |
| 2,363,134 | McCleary          | Nov. 21, 1944 |
| 2,416,265 | Mac Mullen et al. | Feb. 18, 1947 |
| 2,431,011 | Zimmer et al.     | Nov. 18, 1947 |